

Dec. 8, 1942.

C. C. HEIN

2,304,090

COPPER OXIDE RECTIFIER

Filed July 26, 1939

*Fig. 1.*



*Fig. 2.*

WITNESSES:

*C. J. Weller.*

*Henry Diamond.*

INVENTOR  
Carl C. Hein.

BY

*F. W. Lyle.*  
ATTORNEY.

## UNITED STATES PATENT OFFICE

2,304,090

## COPPER OXIDE RECTIFIER

Carl C. Hein, Forest Hills, Pa., assignor to Westinghouse Electric & Manufacturing Company, East Pittsburgh, Pa., a corporation of Pennsylvania

Application July 26, 1939, Serial No. 286,613

9 Claims. (Cl. 148—3)

My invention relates to current rectifying apparatus and has particular relation to rectifiers of the copper-copper-oxide type.

Because of certain inherent physical and chemical properties, the field of use of copper-copper-oxide rectifiers constructed in accordance with the teachings of the prior art is severely limited. A rectifier unit cannot be operated continuously to yield an output potential greater than 3 to 6 volts. Moreover difficulty is encountered in using the rectifiers at elevated temperatures.

It is an object of my invention to provide a copper-copper-oxide rectifier with which output potentials substantially greater than 6 volts shall be attainable.

Another object of my invention is to provide a copper-copper-oxide rectifier that shall operate without difficulty at elevated temperatures.

A further object of my invention is to decrease the space required by a copper-copper-oxide rectifier arrangement for a given rating.

Still another object of my invention is to provide a copper-copper-oxide rectifier of simple structure.

More concisely stated, it is an object of my invention to provide copper-copper-oxide rectifiers that shall function satisfactorily within the range of potentials for which thermionic rectifiers are now used.

My invention arises from the realization that the difficulties encountered in using a prior art copper-copper-oxide rectifier may be primarily attributed to the fact that the element has a negative temperature coefficient. When a rectifier is in operation it conducts substantial forward load current and a small reverse current. An increase in the temperature of the rectifier results in a decrease in both the forward resistance and the back resistance so that when the temperature of a copper-copper-oxide rectifier increases, the forward current and the reverse current also increase. The increased current flow through the rectifier gives rise to a further increase in temperature and the result is that the resistance is further decreased and the current flow still further increased. This continues until the rectifier is damaged or completely destroyed.

On analyzing the negative temperature coefficient, I have come to the conclusion that it arises from the presence of impurities in the copper from which the rectifier is formed. It appears that among the impurities lead is particularly objectionable. The impurities cannot be removed from the element without difficulty. Copper has a relatively low vapor tension so that the impurities

are not easily ejected from its surface. When the copper is heated at atmospheric pressure or in a relatively good vacuum in which the pressure is, for example, of the order of several millimeters, the impurities are oxidized and the undesirable properties of the element are, as a matter of fact, increased.

In accordance with my invention the impurities are removed by heating the copper from which the rectifier is formed in a high vacuum. For the most satisfactory rectifiers, the pressure should be less than .1 micron. At times, however, satisfactory results have been attained with the copper heated in a vacuum having as high a pressure as 30 microns. The heating should be carried out for several hours at a temperature of the order of 1000° C. The temperature should preferably be between 900° C. and 1070° C., the fusing temperature of copper. I have found, however, that heating at 700° C. produces satisfactory results, although the improvement increases with temperature and with the time interval during which the heating takes place.

The novel features that I consider characteristic of my invention are set forth with particularity in the appended claims. The invention itself, however, both as to its organization and its method of operation together with additional objects and advantages thereof will best be understood from the following discussion when read in connection with the accompanying drawing, in which:

Figure 1 shows the improvement attained with a rectifier produced in accordance with my invention; and

Fig. 2 shows an arrangement with which my invention may be practiced.

In the practice of my invention, the principal feature is the heating of the metal in a high vacuum prior to its oxidation. The copper base or blank is initially in the form of a small disc or plate or in the form of a large plate from which a number of small discs or plates are stamped. Whatever the form, the surface is first cleansed of grease by the application of carbon-tetra-chloride. The base is then dipped into concentrated nitric acid, and reused in distilled water. After the acid treatment, the base is disposed in a vessel which is highly evacuated and heated for three hours at a temperature of from 900° C. to 1000° C. The pressure in the vessel is maintained at less than 1 micron and should preferably be less than .1 micron.

During the course of the treatment, the metal gives up a number of impurities in its surface

and particularly lead. The impurities are emitted in a vaporous state, and will, of course, materially increase the pressure. For this reason, it is necessary that the vessel within which the plates are disposed be continuously pumped. While a pressure less than 1 micron has been found to yield the most satisfactory results, I have at times obtained satisfactory rectifiers with the pressure during the treatment somewhat higher. However, in no event should the pressure be greater than 30 microns.

In the customary practice of my invention, the blanks are now oxidized in another furnace. Accordingly, after the three hour treatment, the evacuated container is reduced to room temperature and the blanks are removed and placed in an oxidizing furnace. Here, the blanks are again heated and air or oxygen, preferably at atmospheric pressure, is applied. The oxidizing heating is at a temperature of from 1020° C. to 1030° C. and the treatment continues for 13 minutes. Of course, where convenient, the oxidizing treatment may be carried out in the same furnace as the vacuum treatment. In such a case, it is unnecessary to reduce the blanks to room temperature.

After the 13 minute oxidizing treatment, the blanks are annealed at 500° C. for 13 minutes and then quenched in cold water. The surface of the copper is now coated with a layer which is predominantly cuprous oxide. Whatever cupric oxide happens to be present is now dissolved in the conventional manner and the usual contacts are applied.

A comparison of the characteristics of the vacuum treated copper-copper-oxide rectifier and the present standard rectifier is given in Figure 1. The curves in this view are the result of actual tests carried out with a number of rectifiers. In the upper right-hand quadrant, the current which flows through a short-circuited disc is plotted as a function of the potential for two limiting temperatures, -40° C. and +40° C. Current is plotted vertically in amperes and potential is plotted horizontally in volts. The lower oblique full line curve 3 represents the function at -40° C. for the prior-art standard rectifier. The other oblique full line curve 5 represents the function at 40° C. for the same rectifier. It is to be noted that as the temperature of the rectifier changes the short-circuit current varies over a wide range. The large increase in the current flow for increase in temperature further increases the temperature and tends to produce a run-away effect.

The shaded area 7 between the oblique broken line curves 9 and 11 represents the corresponding range of variation for the rectifier according to my invention. In this case, it is to be noted that the range of variation is materially smaller.

In the lower left-hand quadrant the back current is plotted as a function of the back potential. In this case, current is plotted vertically in milliamperes and potential horizontally in volts. The full line curve 15 which is at a very small angle to the abscissa represents the situation for the prior art rectifier at -40° C. The smooth full line curve 17 extending from the origin represents the situation at 40° C. for the prior art rectifier. The range of variation in the back current is seen to be considerable, and its contribution to the run-away effect is considerably more critical. The broken line curves 19 and 21 bounding the shaded area 23 represent the situation for the rectifier according to my invention -40° C. and 40° C. respectively. It is seen that recti-

5 fiers formed in accordance with the practice of my invention show a vast improvement over prior art rectifiers.

Rectifiers according to my invention are characterized by a substantially greater output and a substantially smaller heating effect than the prior art rectifiers. Because of this, the cooling fins required for the prior art rectifiers for the improved rectifiers designed for the same load are not necessary, and smaller units may be used. The volume requirement of the necessary vacuum-treated rectifiers for a given load may be as much as  $\frac{1}{8}$  of that required for the prior art rectifiers used to supply the same load. Conversely, if the cooling fins are used with the improved rectifiers, and the same number of improved rectifiers as prior art rectifiers are used, the increase in the output rating for the improved rectifiers is 6 to 8 times the output rating of the prior art rectifiers.

My invention also makes possible the use of dry rectifier units at moderately high potentials where appreciable power is required. A rectifier, in accordance with my invention, has been used to supply .7 ampere direct current at 1500 volts continuously. The dimensions of this rectifier are 15" x 15" x 3" and when operated at the aforementioned rating, its efficiency was greater than 80%.

30 Because of the improvement which is introduced by my invention and the saving in cost which is effected, the improved rectifiers may be sold in competition with gaseous or vacuum discharge rectifiers. Over such rectifiers, the copper-copper-oxide rectifiers have a number of marked advantages. For example, the danger of sudden failure by reason of failure of the filament, is absent. No heating time for a filament is necessary. The copper-copper-oxide rectifier is, moreover, a solid object and can withstand shock such as is experienced on board of a battle ship, for example, by reason of gun-fire, better than the glass tube rectifiers.

35 The system with which the vacuum treatment is carried out in accordance with my invention is shown in Figure 2. The copper blanks are, in this case, in the form of plates 25. The blanks are mounted in a rack 27 which is disposed in a cylindrical container 29, preferably composed of a nickel-chromium alloy, sold under the trade name "Nichrome." The cylinder is provided with an opening 31 at one end, through which the rack 27 is inserted and which is closed by a metal plate 33. The neck 35 of the cylinder 29 and the plate 33 are supplied with cooling water 37 which prevents these portions from becoming over-heated.

40 The cylinder 29 is in communication with a suitable vacuum pump 39 through an outlet 41 in the neck 35. The pump 39 may operate alone or a mechanical pump may be interposed in series with it.

45 The temperature of the container 29 and its content is raised electrically by a resistance heater 43 embedded in an insulator 45 which is disposed around the container. To determine the temperature within the container, a thermocouple 47 is provided.

50 While in the preferred practice of my invention the copper blanks are vacuum treated, there are alternative procedures. For example, the copper melt, before being cast into an ingot, may be vacuum treated to produce the desired characteristics. Of course, the vacuum treatment 55 should be the same as in the case of the solid

blank. That is, to say, the pressure should be maintained preferably at less than .1 micron.

Although I have illustrated and described certain methods of treatment in accordance with my invention, I am fully aware that many modifications thereof are possible. My invention, therefore, is not to be restricted except insofar as is necessitated by the prior art and by the spirit of the appended claims.

I claim as my invention:

1. The method of preparing a blank copper disc for oxidation, to produce a copper-copper-oxide disc, which includes the step of heating said blank disc in a vacuum for several hours at a pressure of less than 30 microns and at a temperature of from 700° C. to the fusing temperature of copper.

2. The method of preparing a blank copper disc for oxidation, to produce a copper-copper-oxide disc, which includes the step of heating said blank disc in a vacuum for a time interval of the order of two hours at a pressure of less than 30 microns and at a temperature of from 700° C. to the fusing temperature of copper.

3. The method of preparing a blank copper disc for oxidation, to produce a copper-copper-oxide disc, which includes the step of heating said blank disc in a vacuum for a time interval of the order of two hours at a pressure of less than .1 micron at a temperature of from 700° C. to the fusing temperature of copper.

4. The method of preparing a copper-copper-oxide rectifier disc from a copper disc, which comprises the steps of cleansing said copper disc to remove grease and the like from the surface, heating the cleansed copper disc for a time interval of the order of three hours at a temperature of from 700° C. to the fusing temperature of copper in a vacuum at pressure of less than 30 microns thereafter heating the copper disc in

an oxidizing atmosphere at a temperature of 1020° C. to 1030° C. for a time interval of the order of 13 minutes, annealing the disc thus oxidized by heating at 500° C. for a time interval of 5 the order of 13 minutes and quenching the annealed disc in a cold fluid.

5. In the production of a copper-copper-oxide rectifier disc, the method of preparing a blank copper disc for oxidation which includes the step 10 of heating said blank copper disc in a vacuum for a time interval greater than one hour at a pressure of less than 30 microns and at a temperature of from 700° C. to the fusing temperature of copper.

15 6. In the production of a copper-copper-oxide rectifier disc, the method of preparing a blank copper disc for oxidation which includes the step of maintaining the melt from which the blank copper discs are to be formed at a pressure of 20 less than 30 microns for a substantial time interval.

7. The process of producing copper-oxide rectifier elements which comprises the steps of vacuum-treating molten copper, congealing said 25 copper, and subsequently oxidizing its surface.

8. The process of producing copper-oxide rectifier elements which comprises the steps of vacuum-treating molten copper in an enclosure which has been exhausted to a pressure not exceeding the order of 30 microns, congealing said 30 copper, and subsequently oxidizing its surface.

9. In the production of a copper-copper-oxide rectifier disc, the method of preparing a blank copper disc for oxidation which includes the step of heating said blank copper disc in a vacuum for a time interval at least of the order of one hour at a pressure of less than 30 microns and at a temperature of from 700° C. to the fusing 35 temperature of copper.

CARL C. HEIN.